

## UNITED STATES PATENT OFFICE

WILLIAM H. BASSETT, OF CHESHIRE, CONNECTICUT, ASSIGNOR TO THE AMERICAN BRASS COMPANY, OF WATERBURY, CONNECTICUT, A CORPORATION OF CONNECTICUT.

## ALLOY WIRE

No Drawing.

Application filed June 18, 1928. Serial No. 286,489.

This invention relates to a metal alloy and conductor wire manufactured therefrom, and has for an object to produce an alloy wire which will have the required strength, ductility and the electrical conductivity for use 5 for twisted pair drop wire or lead-in wire such as is used for telephone installations, although it is not necessarily limited to this use. A copper clad steel wire has been used for this purpose as it has a conductivity which 10 was quite satisfactory and the required strength, but it has a serious objection in that it lacked uniformity, and considerable experimentation has been carried on to discover an alloy which could be easily drawn to 15 the required size and which would have the required strength, resistance to shock and electrical conductivity.

After considerable experimentation I have 20 developed an alloy which can be drawn to the proper size and will have the required strength, conductivity, and resistance to shock to meet the standards set. This is an alloy of cadmium, zinc and copper, the 25 portions of cadmium ranging from about  $\frac{1}{2}$  to about  $1\frac{1}{2}\%$ , zinc from about 2 to about 7% and the balance copper. In manufacturing this alloy and wire the commercial practice of casting the material into an 30 approximately 200 pound bar, and approximately four inch square cross section was used. The bar after gating was heated in a muffle and hot rolled to approximately  $\frac{1}{2}$  inch diameter and then drawn through dies 35 on the standard type of continuous wire drawing machine to .045 inch diameter.

This wire is very satisfactory for the purpose intended as it has a conductivity of approximately 55% based on the international annealed copper standard at  $20^{\circ}$  C., and it has the required tensile strength, meeting the breaking strength requirement of 170 pounds for the .045 inch diameter of hard drawn wire. The conductivity of the wire 45 and the exact strength obtained following a definite amount of cold working depends, of course, upon the amount of cadmium and zinc which is introduced into the alloy. The material containing the smaller amounts of 50 cadmium and smaller amounts of zinc will

have a higher conductivity and lower strength than the material which contains a relatively large amount of cadmium and a larger amount of zinc. This alloy gives a wire which is especially adapted for use in the manufacture of drop wires or leading-in wires which are strung by the utility companies (telephone or telegraph) between their cables and the subscriber's building. This wire is fairly strong, approximately 55 120,000 pounds per square inch tensile strength, and is not easily broken down by a falling limb or a sudden loading of the wire in an ice or sleet storm, or by the strains 60 set up in the wire due to high winds.

The wire after being drawn to size may be wound on a reel and then passed through a flux and through molten tin, wipes and water to give a satisfactory tinned surface. Tin 65 on the wire is required in order to protect the material from the rubber and insulating materials which are applied to the wire by the insulating companies.

Having thus set forth the nature of my invention, what I claim is:

1. A metal alloy comprising from about 70 one half to about one and one half per cent cadmium, from about two to about seven per cent zinc, and the balance copper.

2. A drawn metal wire comprising from 75 about one half to about one and one half per cent cadmium, from about two to about seven per cent zinc, and the balance copper.

3. A metal conductor wire comprising an 80 alloy of cadmium, zinc and copper, having from about one half to about one and one half percent cadmium, from about two to about seven percent zinc, and the balance copper, and having an electrical conductivity of approximately 55 per cent or greater based on the international annealed copper standard at  $20^{\circ}$  C., and capable of being drawn to have a tensile strength of at least 85 about 120,000 pounds per square inch.

In testimony whereof I affix my signature.

WILLIAM H. BASSETT.